

# United States Patent Office

3,444,120

Patented May 13, 1969

1

3,444,120

## GLASS FABRIC HAVING IMPROVED YARN SLIPPAGE AND HAND

David W. Boyes, North Scituate, and Douglas E. Potter, Cumberland, R.I., assignors to Owens-Corning Fiberglas Corporation, a corporation of Delaware  
No Drawing, Filed Mar. 14, 1966, Ser. No. 533,804  
Int. Cl. C03c 25/02; D06c 25/00  
U.S. Cl. 260—29.6

7 Claims

### ABSTRACT OF THE DISCLOSURE

A liquid treatment for fibers, and particularly glass fibers, which provides improved "hand" and high retention of the strands against edgewise removal.

The present invention relates to a coating material for glass fibers which will produce a durable smooth finish and will flexibly bond adjacent fibers together; and to glass fibers and woven glass fabrics so coated.

Prior to the present invention, it has not been possible to produce flexible glass fabrics whose fibers could not easily be pulled from a cut edge. The art commonly calls endwise removal of fibers from a cut edge "yarn slippage". "Yarn slippage" is measured by an ASTM test procedure D434-42. According to this test procedure, a 4" x 4" piece of glass fabric to be tested is sewn onto a 4" x 8" piece of the woven fabric using fourteen stitches to the inch, and the force required to pull the piece of cotton fabric from the fabric being tested using a Scott Tester is recorded in pounds and is directly proportional to the force required to remove the fibers endwise from the fabric. The greater the numerical value of yarn slippage, the stronger the fabric. The "hand" of the fabric is a term used to describe the flexibility of the fabric and is arbitrarily determined by wadding the fabric up in a person's hand. The ease by which the wadding takes place is termed the "hand" of the fabric, and the softer or more flexible the fabric, the better the "hand." A coating which cracks during the wadding process, is unacceptable for textile uses.

Prior to the present invention, there were no finished coatings for glass fibers which would produce a fabric of acceptable "hand" comparable to that of cottons, woolens, and the like, and which would have a high numerical value of yarn slippage. Heretofore, resin binder finishes which would bind smooth glass fibers together in a manner providing high "yarn slippage" were too stiff to provide good hand. Conversely, binder coatings which were sufficiently flexible to provide a good hand for glass fabrics were not sufficiently strong to give high numerical values of yarn slippage. The problem has been a difficult one and has prevented glass fabric from being used in many textile applications, as for example blankets, wearing apparel, and other materials which are washed frequently. In addition to withstanding the flexing and abrading that occurs during washing operations, the finished coating must be water insoluble, it must prevent the water from penetrating to the surface of the glass, and it must in most cases be capable of fixing organic and/or inorganic dye stuffs so that they will not be removed during washing.

An object of the present invention is the provision of a new and improved finish coating for glass fabrics which will provide high yarn slippage and good hand.

A further object of the invention is the provision of a new and improved coating for glass fabrics which will provide high yarn slippage, good hand, and which coating will not be removed by repeated machine washings using water and detergent.

2

A further object of the invention is the provision of a new and improved finished coating material of the above described type which will permanently fix organic and/or inorganic pigments or dyes to glass fabric.

Further objects and advantages of the invention will become apparent to those skilled in the art to which it relates from the following description of the structure produced by the invention as well as preferred embodiments, and the manner in which these embodiments are made.

The finished coatings which have been used heretofore have generally been polymeric materials which have been polymerized in situ to provide a generally impervious resin coating bonded to the glass fibers. These coatings have sometimes been laid down from organic solution while others have been laid down from water emulsions. In either instance, sufficient polymerization has taken place to provide a stiff polymer layer. Some of these films have depended upon continuity about the glass fibers for affecting a bond to the fibers, while others have used bonding agents such as organosilanes or organo metal complexes to chemically attach the coatings to the surface of the glass fibers.

It has now been discovered that it is possible to produce an impervious coating having good hand and yarn slippage, as well as all of the other necessary properties of a good textile finish, by a structure wherein particles of a resin are mechanically interlocked in a film with some of the interlocking particles being connected to one glass fiber while others are connected to an adjacent glass fiber. Weak secondary forces bond the particles of the resin together to provide an impervious finish layer while permitting a relative flexure of the particles, and chemical bonds bind the particles to the glass. Because the particles are interlocked, relatively high tensile strength is produced; and because the particles are not bound together by strong primary chemical bonds, the film has good flexibility.

A desirable interlocking of the resin particles is achieved by chemically bonding one functional group of a water soluble bi-functional molecule to a particulate matter supported as a water emulsion or dispersion, and bonding the other functional group of the molecules to the surface of the glass. Upon removal of the water, the resin particles become mechanically knit together, and because of their hydrophobic nature will generally exclude water. While some cross-linking of these particles of polymer may take place, secondary forces such as Van der Waal forces will hold the film together to produce a very flexible yet strong film. Where increased stiffness is desired, particles of a polymer having some remaining reactive groups can be used to provide a small amount of chemical cross-linking between the particles at locations where they are brought together during the removal of the water. This cross-linking, of course, will not be complete so that relative rotation of these particles can still take place. The structure can be likened to a plurality of interlocking balls which are free to rotate relative to each other and are sufficiently close to each other to prevent an inside layer of the balls from being pulled outwardly of an outer layer of the balls. Molecular handles of sufficient length, extend between the outer balls to attach the inside balls to a glass surface outwardly of the outer balls.

The invention is best exemplified by the following preferred embodiment.

#### Example 1

A textile fabric of glass fibers is heat cleaned to remove any previous size and is then immersed for five

minutes in a water system containing approximately 12 percent by weight of the following mixture of ingredients.

| Ingredients:                      | Parts by weight |
|-----------------------------------|-----------------|
| Soluble epoxy prepolymer (solids) | 0.5             |
| Acetic Acid                       | 0.05            |
| Syl-Soft 16 (solids)              | 3.0             |
| Polycryl 7F12 (solids)            | 4.0             |
| Polycryl 7F10 (solids)            | 2.5             |
| Aridye Padding N Colors           | 2               |

"Polycryl 7F12" is a trade name of Polymer Industries, Inc. for an emulsion of a polyacrylic acid polymer having substantially no remaining active groups except carboxyl groups. "Polycryl 7F10" is a trade name of Polymer Industries, Inc. for an emulsion of an acrylic material containing an acrylic copolymer polymerized to a high molecular weight material having some amine and carboxyl groups remaining. "Syl-Soft 16" is a trade name of Dow Corning Corp. for a copolymer of methyl hydrogen silicone and dimethyl silicone having some labile hydrogen remaining. Aridye Padding N Colors are made by Inter-chemical Corporation. The water soluble epoxy is a material produced in accordance with U.S. application, Ser. No. 213,133, filed July 30, 1962 and continuation-in-part Ser. No. 540,532, filed Apr. 6, 1966, now U.S. Patent 3,336,253. This material has a substituted ammonium ion at one end of a molecular chain with an oxirane group spaced therefrom by more than approximately ten atoms. The epoxy material before reaction with the amine had the following formula:



Some lower polymers of the above molecule were also present in the material.

A hundred pound mix of the material is prepared by mixing 0.05 pound of glacial acetic acid to 1.0 pound of the epoxy material dissolved in diacetone alcohol followed by the addition of two pounds of warm water added slowly while stirring until the epoxy material goes into solution. This material is put into a mix tank containing 10 pounds of water, and the alkyl hydrogen silicone (Syl-Soft 16) is added thereto and thoroughly mixed. Thereafter, emulsions of the polyacrylates (Polycryl 7F12 and Polycryl 7F10) are added with stirring. The dye stuff is added and thereafter sufficient water is added to make a hundred pounds of the mix. In those instances where an anionic dye stuff is used, the pH is first raised to 8 with ammonium hydroxide. A fabric weighting 4.76 ounces per square yard having a warp of 60 yarns per inch, and a fill of 58 yarns per inch when immersed in the above material and dried at 350° F. will have a coating comprising between 1½ to 2% by weight of the finished cloth as determined by ignition loss and will have an ASTM yarn slippage value of from 30 to 35 pounds. This material will withstand ten machine washings without apparent loss of color.

The water soluble epoxy prepolymer used in the above example is a long chain molecule having two functional groups separated by a chain of at least ten atoms. As explained in the application, Ser. No. 213,133, long chain otherwise insoluble molecules, whether or not they include oxirane groups, can be water solubilized by a substituted ammonium ion having OH groups in proximity thereto. The combination of the OH group and the ammonium ion in combination produces a very strong solubilizing affect. In the materials taught by application Ser. No. 213,133, the OH groups are attached to the beta carbon relative to the nitrogen atom, and this OH group provides one functional group of the difunctional solubilized molecule. Where the solubilized molecule is an epoxy, it will, of course, have an oxirane group as the other functional group, and this is located in the chain more than ten atoms away from the OH group.

In general the hydrogen of a primary or secondary amine is more reactive than an OH group on a carbon atom, and an OH group is more reactive than a carboxyl group. In the particular materials of the above identified application the OH group is believed to be selectively reacted with the hydrolyzed hydrogen site of the silicon atom of the organo-siloxane because the ammonium ion adjacent thereto is cationic, and this charge phenomenon draws this end of the molecule toward the hydrolyzed silicon atom. The reaction between the OH group and the hydroxyl site of the silicon atom to form a C—O—Si bond can proceed either immediately or over a period of time depending upon temperature, because the molecules are held in an oriented position. When the polyacrylic polymers are added to the mixture, the oxirane groups are therefore in the vicinity of the carboxyl groups of the polyacrylic acid, and a reaction there between takes place when the coated fabrics are dried at approximately 350° F.

The Polycryl 7F12 material used in the above example is a polymer of medium molecular weight whose remaining reactive groups consist principally of carboxyl groups. While this material can be linked to other functional groups, such as the oxirane group of the water soluble molecules used in Example 1, it will generally be desired to produce a stronger bond relative to the water soluble molecules. This can be conveniently accomplished by using a polyacrylic acid containing additional, more reactive groups, such as amine groups. The Polycryl 7F10 is such a material and will cross link more easily and quickly to the water soluble molecules during the time that the water is being evaporated, and during the time that the film on the fabric is shrinking together. It has been found, however, that the use of the more reactive 7F10 by itself produces too much cross linking between the polymer particles. By disbursing the more reactive 7F10 particles among 7F12 particles the cross linking of these particles is greatly reduced without decreasing the strength of its chemical bonds to the long chain water soluble molecules. Because the water soluble molecules of Example 1 have different functional groups at its opposite ends, only one functional group of each molecule is caused to react with the organo-siloxanes, and substantially no cross linking is produced at this time. Thereafter the other functional group, which is less reactive, can be caused to react selectively with the later applied particles.

After the molecules have been linked up in the selective manner above described, a dye stuff is added which will react with remaining functional groups, or as in the case of inorganic pigments, is mechanically bound during the shrinkage that takes place during the drying and curing stage. These dye stuffs can be non-ionic or cationic in nature, and if the bath into which the fabric is dipped is caused to have a pH greater than approximately 8, as produced by the addition of ammonium hydroxide and the like, an anionic dye can be used. The dyes which can be used, although not limited to, may include: nitroso pigments such as Naphthol Green B; nitro pigments such as Naphthol Yellow S, Pigment Chlorine GG and Lithol Fast Yellow GG; azo pigments such as Toluidene red, para reds, hansa yellows, permanent orange, benzidene yellows, Persian orange and Lithol red; pyrazolone pigments such as Hansa Yellow R; basic dye pigments such as Malachite Green, Crystal Violet, Auromine O, Auromine G, Setoglaucine, Brilliant Green, Magenta, Methyl Violet, Rhodamine B, Thioflavin T, Methylene Blue; auxanthine dye pigments, anthroquinone pigments, vat color pigments and phthalocyanine pigments such as indigo, Ciba Violet, Algal Yellow, Monastral Blue, Syrian Blue and the like.

After a film of the material given in Example 1 has been formed, it may be desirable in some instances, although not necessary, to apply a water proofing, and/or a material which will aid in fixing some of the dye stuffs, as is well known in the art. In some instances, it may be desirable to apply a 2 to 2.5% solution of Quilon which is a chromium organo complex commonly used as a final water proofing treatment.

